

## UNITED STATES PATENT OFFICE

FRANCIS J. CURTIS, OF BELMONT, MASSACHUSETTS, ASSIGNOR TO MERRIMAC CHEMICAL COMPANY, INC., OF BOSTON, MASSACHUSETTS, A CORPORATION OF MASSACHUSETTS

## METHOD OF SIZING FIBROUS MATERIAL

No Drawing.

Application filed August 10, 1929. Serial No. 385,084.

My invention relates to sizing fibrous material, particularly, but not exclusively, cellulose fibers, and is particularly useful in the production of paper products.

The invention, which has among its objects increasing the durability of paper or the like, will be best understood from the following description of a process of making paper constituting one embodiment of the invention, while the scope of the invention will be more particularly pointed out in the appended claims.

Heretofore, paper commonly has been made by beating cellulose fibers in a beater to which is added rosin size, the latter commonly made by boiling soda ash and rosin and atomizing the solution in water. After the mixture has been beaten for a requisite length of time, suitable for the grade and kind of paper being made, and just before the end of the beating operation, alum is added, and the beaten mixture is poured from the beater, given further mechanical treatment, and finally, after dilution, is made into paper by use of a Fourdrinier or cylinder machine. Commonly about  $1\frac{1}{2}$  pounds of alum to each pound rosin equivalent of the rosin size are necessary to secure proper sizing.

As is well known by those skilled in the art, paper made according to the above described prior process lacks durability in the sense that it is subject to chemical deterioration. This deterioration is believed to be largely due to the acidity of the paper pulp consequent upon the addition of the necessary amount of alum to secure effective sizing. It has been found that the mixture of cellulose fibers and rosin size is very alkaline, commonly having a hydrogen ion concentration equivalent to a pH value of 9 or 10, or even more. The addition of the requisite amount of alum to secure proper sizing, it has been found, commonly reduces the pH value to somewhere around 4.5 to 4.8, which indicates considerable acidity. It is believed that the phenomenon, which occurs in this prior process, is that the alum in solution dissociates into sulphuric acid and colloidal alumina, the sulphuric acid acting to

precipitate the rosin from the size, and the colloidal alumina forming a so-called "colloidal complex" between the alumina, cellulose, and rosin, it being understood that colloids having the same electrical charge 55 will not unite in the absence of a bond having an opposite electrical charge, and that the cellulose and rosin colloids both have a negative electrical charge which will prevent their cementing in the absence of the 60 colloidal alumina which has a positive electrical charge. It has been found that if the sized pulp has an acidity indicated by a pH value which is not lower than about 6 the paper produced is not subject to chemical 65 deterioration, but that in most instances, if only sufficient alum is added to secure this pH value, improper sizing will result, the sizing in such cases being due merely to a mechanical mixture of the precipitated rosin 70 and cellulose fibers. Therefore, it is necessary, in the prior process, to use sufficient alum to supply the necessary amount of colloidal alumina to secure effective sizing, with the result that the pH value of the 75 pulp is reduced to a value at which chemical deterioration of the sized paper occurs.

According to the improved process, the requisite amount of colloidal alumina is provided in substantially alkaline combination 80 as distinguished from acid combination. It has been found that the pH value of the pulp may be controlled within any desired limits, while securing sufficient alumina to effect proper sizing, by reducing the amount 85 of alum added to the pulp according to the prior process, and using sodium aluminate for increasing the amount of alumina above that provided by the alum. Preferably, enough alum is added to give the necessary 90 acidity to precipitate the rosin from the alkaline rosin size, the remaining necessary alumina being provided by the sodium aluminate. With the improved process, by varying the proportions of alum and sodium aluminate, any desired pH value of the pulp and amount of alumina therein may be secured, whereas with the prior process, increasing the amount of alumina necessarily increases 95 the amount of acid present, with the result 100

that when proper sizing is effected by the prior process, the pH value is so low that the paper produced and the machinery employed for producing it, particularly the expensive wire belts, are subject to chemical deterioration, which materially reduces the life of both the paper and said machinery.

The relative amounts of alum and sodium aluminate can be varied within wide limits, depending upon the condition of the paper pulp and the kind and grade of paper produced. When making paper, the alum and sodium aluminate preferably are added in aqueous solution, and preferably at the same time, but to prevent flocking, the two solutions are not mixed before adding them to the pulp.

As one example of the practice of the method, but without limitation thereto, I have found that satisfactory results can be obtained, when using standard sulphite pulp beaten with 2% by weight of rosin, the latter in the form of the above described rosin size, by adding alum



and sodium aluminate ( $\text{Na}_2\text{O} \cdot \text{Al}_2\text{O}_3$ ) in the ratio of 3:1, with the total alumina ( $\text{Al}_2\text{O}_3$ ) the equivalent of 3% of alum based on the weight of pulp. With this mixture sizing is obtained, at a pH value of 6.5, as satisfactory as that obtained by use of alum alone at a pH value of 4. In practice, the character of the pulp and amount of rosin employed vary widely according to the kind and grade of paper to be made. In practising the invention the necessary amounts of alum and sodium aluminate may be determined for given conditions by gradually adding alum to the first beater handling the material, and continually testing samples of the liquor for pH value until a pH value is obtained which indicates the rosin is precipitated. Commonly for usual rosin size this pH value will be about 5, but for any rosin size the value can be readily determined by previous sample tests. After precipitation of the rosin, sodium aluminate may be gradually added to the beater until tests of samples of liquor drawn from the beater indicate the desired pH value of the pulp. Preferably a final pH value of about 6.5 is secured, but good results will be obtained with pH values between 5 and 7. It will be understood that the pH value of the samples of liquor may be quickly obtained by use of any of the several known electrometric or colorimetric methods.

As substitutes for the specific rosin size hereinbefore mentioned other forms of colloidal rosin, starch, glue, and other negatively charged colloids, may be employed, and the invention is applicable to soda and other

pulps commonly employed in the art as well as to sulphite pulp.

It will be understood that wide deviations may be made from the examples of the invention herein described without departing from its spirit.

I claim:

1. The process of cementing negatively charged colloidal size to the cellulose fibers in a mixture of the two which comprises adding alum and sodium aluminate. 75

2. The process of sizing cellulose and like fibers which comprises mixing said fibers with rosin size, precipitating the rosin by adding alum to the mixture, and controlling the pH value of the mixture by adding sodium aluminate thereto. 80

3. The process of sizing cellulose and like fibers which comprises mixing said fibers with rosin size, precipitating the rosin by adding alum to the mixture, and augmenting the amount of alumina provided by the alum and controlling the pH value of the mixture by adding sodium aluminate. 85

4. The process of producing sized paper products which comprises beating cellulose fibers with rosin size, precipitating the rosin in the beaten mixture by adding alum, and controlling the pH value of the mixture by adding sodium aluminate thereto. 90

5. The process of producing sized paper products which comprises beating cellulose fibers with rosin size, precipitating the rosin by adding alum to the beaten mixture, and augmenting the amount of alumina provided by the alum and controlling the pH value of the mixture by adding sodium aluminate. 100

6. The process of producing sized paper products which comprises beating cellulose fibers with rosin size, and afterward beating the mixture with sufficient alum for precipitating the rosin and a material amount of sodium aluminate. 105

7. The process of sizing cellulose fibers and the like which comprises beating said fibers with rosin size, adding alum to the beaten mixture to precipitate the rosin with production of colloidal alumina and sulphuric acid in fixed ratio, and controlling the alumina-sulphuric acid ratio by addition of sodium aluminate. 110

In testimony whereof, I have signed my name to this specification.

FRANCIS J. CURTIS.

120

125

130